

## UNITED STATES PATENT OFFICE

2,065,175

## MANUFACTURE OF ARTIFICIAL SILK

Otto Eisenhut, Heidelberg, Hanns Rein, Hamberg von den Hohe, and Erich Kaupp, Ludwigshafen-on-the-Rhine, Germany, assignors to I. G. Farbenindustrie Aktiengesellschaft, Frankfort-on-the-Main, Germany

No Drawing. Application October 9, 1934, Serial No. 747,646. In Germany October 10, 1933

## 6 Claims. (Cl. 18—54)

Our present invention relates to the manufacture of artificial silk and more particularly to the manufacture of artificial silk from viscose.

One of its objects is a process of spinning artificial silk from viscose which is efficient and permits to produce artificial silk at reduced costs. Another object is to produce artificial silk from viscose which has the character of artificial silk produced according to the copper ammonia process. Still another object is the threads produced according to our new process which have the character of copper ammonia silk though spun from viscose. Further objects will be seen from the detailed specification following hereafter.

When it is attempted to make thread from normally ripened or unripened viscose with the use of water as the first precipitating bath, there is difficulty in obtaining a thread having the properties necessary for good artificial silk. This difficulty is encountered in the entire normal range of ripeness of the viscose, that is to say from high salt points to the lowest usual salt point.

We have found that viscose can be spun without troubles into water as a first precipitating bath, for instance, while using a spinning funnel, if the viscose is ripened below the usual ripeness corresponding with ammonium chloride number of 7 to 6 (Hotterroth number).

At normal temperature, a few days elapse between the time when the viscose has the lowest stage of ripeness (which can be determined by the usual measuring methods) and the time when the viscose spontaneously coagulates; the state of ripeness of the viscose solution, which increases during this lapse of time, can be followed exactly and fixed chronologically. The spontaneous coagulation point generally occurs, at a ripening temperature of 20° C., at about 7 days after the above ripeness has been attained.

There is no objection to the acceleration of the degradation of the xanthate molecule by raising the temperature.

When spinning is conducted in the interval of time between the ammonium chloride number 7 to 6 and the spontaneous coagulation (which naturally must be avoided) the viscose is degraded to such an extent that it may be coagulated by water alone or by unusually strongly diluted electrolyte solutions. Such solutions of electrolytes are those which have a precipitating power at most equal to that of an aqueous solution of 1% of sodium sulfate and 0.2% of sulfuric acid. The concentration of the electrolyte in the precipitating bath obviously varies with the spinning con-

ditions and the particular viscose to be spun. The most suitable composition will easily be found by a few comparative experiments. It may also be advantageous, to use a solution which contains only salt or only acid as a precipitating bath, however, as a rule a solution containing salt and acid is preferred. The coagulation may be carried out either in a spinning funnel or in an open bath. The coagulation can also be completed subsequently by means of strongly diluted acid or salt solution or both. The consumption of water is slight; it amounts approximately to ½—1.0 cbm. of cold water per kilo of silk.

Any titer may be spun by this process, to which any cellulose can be subjected, but for which the use of little degraded cellulose is preferred. The use of little degraded cellulose involves the advantage that the thread obtained has a high viscosity and is sparingly soluble in solutions of alkali. The speed of spinning may amount to 80 m. and more per minute; in particular, when the temperature of the water is raised the speed of draft can be increased. The same result can be obtained when spinning with cold water if unusually long precipitating baths (funnels) are used. For instance, when spinning a thread having a single titer of 3 deniers and a total titer of 300 deniers, the length of the spinning funnel is about 50 to 60 centimeters. In general the length of the spinning funnel must be greater when spinning a higher titer and vice versa.

The effect of the extraordinarily unstable condition of the viscose molecule in the vicinity of the spontaneous coagulation point, and the merely slight chemical attack necessary for full decomposition of the much degraded xanthate molecule is that the thread material separated in the precipitation of the cellulose is very similar to the material obtained by the copper silk process. The precipitation is preferably carried out in a spinning funnel. The thread is soft to the touch, the cross-sections are round, that is to say similar to those of copper silk, the tensile strength varies between 140 and 200 grams per 100 deniers, and the extension between 12 and 20 per cent and more. The capacity of the material for being dyed is at least as strongly substantive as that of normal copper silk. Thus, the capacity of copper ammonia silk and of the material according to this invention for being dyed with Diamin-Pure Blue FF (cf. Schultz Farbstofftabellen, 6th edition (C) 424) without the addition of salt, is the same, while the usual viscose silk is hardly dyed by this dye without the addition of salt. The material according to this invention shows

the same structure as copper ammonia silk when investigated by X rays. The material is soft to the touch, is warm and woolly, that is to say is similar to copper silk in this respect also. The 5 material according to this invention differs from copper ammonia silk in that it contains no traces of copper. That the artificial threads made according to this invention are produced according to the viscose process is evident from the fact 10 that they still contain in the finished condition traces of sulfur which can be detected by a sufficiently sensitive method for detecting sulfur.

The following examples illustrate the invention:

15 *Example 1.*—Viscose containing 7.5 per cent of cellulose, 8 per cent of NaOH and which has been sulfidized with 31.5 per cent of CS<sub>2</sub> calculated on the quantity of cellulose from which is started, is stored after having attained the normal ammonium chloride number of 6, for a further three days at 20° C.; it is then passed under a pressure of 8.5 atmospheres, through a spinning head having 92 holes (individual hole diameter about 0.8 mm.) into a spinning funnel, 20 through which flows a slow stream of water at 20° C. A normal coagulation occurs. The thread formed, after leaving the funnel, is passed over a roller or a rod and conducted through a trough through which a dilute acid or a salt solution or 25 a solution of acid and salt flows. There may be used, for example, a sulfuric acid of 3.5 per cent strength in which 6 per cent of sodium sulfate is dissolved. The solution can be used in circulation while keeping its composition and concentration constant. The reeling occurs at a distance of 1/2-1 m. from this trough. The speed 30 of draft is 80 m. per minute. The spun material (titer 140) is then after-treated in normal manner. The thread is strongly substantive in dyeing, is of round cross-section, and is soft to the touch.

35 *Example 2.*—Viscose prepared as described in Example 1, is coagulated in a spinning funnel into an aqueous solution containing 0.5 per cent of Na<sub>2</sub>SO<sub>4</sub> and 0.025 per cent of H<sub>2</sub>SO<sub>4</sub>. The coagulated thread is guided over a roller or a rod and passed through a bath of 10 per cent of sulfuric acid and 3 per cent of sodium sulfate. The 40 supply of the spinning liquid and the other spinning conditions are so selected that a thread with a total liter of 120 deniers and a single titer of 1.3 deniers is formed. The resulting thread of which the filaments are well closed and have a round cross-section, has a tensile strength in the dry state of 203 grams per 100 deniers and an extensibility of 14.6 per cent. It possesses the dyeing properties of copper ammonia silk.

45 *Example 3.*—Viscose containing 7.5 per cent of cellulose and 7 per cent of NaOH which was stored for three days at 20° C. after having reached the normal Hottenroth degree of 6, is pressed at 8.5 atmospheres through a spinning head with 90 openings of 0.8 mm. diameter each 50 into a spinning funnel through which flows slowly a current of water of 14° C. The rate of viscose supplied per minute is regulated so that at a speed of draft of 40 meters per minute there is produced a single titer of 0.47 deniers. After 55 leaving the funnel the thread is guided through a channel. Through this channel flows sulfuric

acid of 10 per cent strength containing 3 per cent of sodium sulfate. The tensile strength of the thread which has the dyeing properties of copper ammonia silk and the filaments of which are well closed, amounts to 212 grams per 100 deniers and 60 the extensibility to 11.3 per cent.

The spinning temperature depends upon the single titer which is spun and the degree of ripeness of the viscose. The higher the single titer the higher is the spinning temperature the remaining conditions of operation being the same. For instance, when using Permutite-water having a carbonate hardness of 1.5 and spinning a single titer of 3 deniers with a viscose having a degree of ripeness of 1.5 through a spinning funnel of 60 10 centimeters length at a speed of draft of 60 meters per minute, a spinning temperature of 25° C. has been found to be suitable. These statements are however not intended to limit the invention, but the most suitable spinning conditions 15 in each particular case will be found by a few comparative experiments.

What we claim is:

1. A process of manufacturing artificial silk from viscose which comprises squirting viscose 20 having a degree of ripeness below 7 to 6° Hottenroth through the openings of a spinning nozzle into water.

2. A process of manufacturing artificial silk from viscose which comprises squirting viscose 25 having a degree of ripeness below 7 to 6° Hottenroth through the openings of a spinning nozzle into water, and passing the formed threads through a hardening bath.

3. A process of manufacturing artificial silk 30 from viscose which comprises squirting viscose containing 7.5 per cent of cellulose and 8 per cent of NaOH, and which after having reached the Hottenroth degree of 6 has been stored for three 35 days at 20° C. through a spinning head having openings of 0.8 mm. diameter each, into a spinning funnel through which flows a slow stream of water of 20° C., and hardening the formed threads in sulfuric acid of 3.5 per cent strength 40 containing 6 per cent of sodium sulfate. 45

4. A process of manufacturing artificial silk from viscose which comprises squirting viscose containing 7.5 per cent of cellulose and 7 per cent of NaOH, and which after having reached the Hottenroth degree of 6 has been stored for 50 three days at 20° C. through a spinning head having openings of 0.8 mm. diameter each, into a spinning funnel through which flows a current of water of 14° C. and hardening the formed threads in a bath of 10 per cent of sulfuric acid 55 and 3 per cent of sodium sulfate.

5. Artificial threads consisting substantially of cellulose hydrate, having the capacity of being 60 strongly dyed by Diamin-pure blue FF without the addition of salt, but containing in the finished condition no traces of copper.

6. Artificial threads consisting substantially of cellulose hydrate having the capacity of being 65 strongly dyed by Diamin-pure blue FF without the addition of salt, and containing in the finished condition traces of sulfur, but no trace of copper.

OTTO EISENHUT.

HANNS REIN.

ERICH KAUPP.

70